

## UNITED STATES PATENT OFFICE

WILLIAM D. GREEN, OF BAUER, UTAH, ASSIGNOR TO COMBINED METALS REDUCTION COMPANY, OF STOCKTON, UTAH, A CORPORATION OF UTAH

## PROCESS FOR THE EXTRACTION OF RESIN FROM COAL

No Drawing.

Application filed April 19, 1929. Serial No. 356,623.

There are certain coals which contain a valuable resin. Heretofore, it has been proposed to extract the resin by means of solvents such as benzol. This method is expensive and wasteful of the solvent used. It has also been proposed to separate the resin from the coal by use of liquids with high specific gravities. The contamination of the products and mechanical losses of the liquid used make a procedure of this kind expensive.

This invention is based upon the discovery that the relative flotability of resin is enough greater than that of coal that the resin can be effectively floated from coal by a suitable flotation agent such as one of the "higher" alcohols, turpentine, cresol, or one of the pine oils, or the like.

I have found that amyl alcohol is particularly advantageous as the frothing agent for the separation of resin from coal, although other recognized frothing agents may be used. I find that amyl alcohol gives a cleaner resin and a better recovery than the other frothing agents named.

I have also found that the resin froth concentrate produced by using one of these frothing agents contains appreciable quantities of finely divided coal which lowers the grade of the resin, and if the resin is re floated in the presence of a small amount of potassium alum most of this finely divided coal can be eliminated and a high grade resin obtained. The highly concentrated resin so obtained can now be dissolved in suitable solvents for making varnish or lacquer or for other purposes and the resin solution further purified by centrifugal separation, filtering or other means.

The invention involves treating the resin-carrying coal, reduced to a floatable size, i. e., of a size sufficiently fine to liberate the resin from the coal, and in the form of a water pulp with a small quantity of amyl alcohol or other frothing agent in a flotation machine

or apparatus, whereupon the resin collects in the form of a froth and can be removed in the usual manner.

The coal remains in the pulp as the tailing and can be recovered and used as powdered coal.

The resin froth which carries some very finely divided coal can be mixed with a suitable quantity of water, a small quantity of potassium alum added and the resin re floated in another flotation machine or apparatus thus making a clean resin, the finely divided coal remaining in the pulp as tailing.

In carrying out the invention, it is preferable to use cold water because amyl alcohol is a solvent for resin and its solvent action is facilitated by heat, although this is not a necessary limitation of the invention.

The following example illustrates the practice of the invention:

500 grams of resin-bearing coal from Salina Canyon, Utah, was ground with 2 parts of water to approximately pass a 40-mesh screen, which in this case was sufficiently fine to liberate the resin from the coal. An additional quantity of water, sufficient to give a 1:3 pulp, was added and the pulp introduced into a froth flotation machine. Here amyl alcohol was added in the proportion of 0.6 pound per ton of resin-bearing coal and the whole agitated in the usual manner. A froth formed which carried the greater portion of the resin and was removed, the coal remaining in the pulp as a tailing.

The resin froth was now prepared for and subjected to selective flotation treatment that is, the resin froth was introduced into a flotation machine, water added in sufficient quantity to fill the machine to working level, 0.4 pound of potassium alum per ton of original resin-bearing coal was added, the whole agitated, then 0.2 pound of amyl alcohol per ton of original resin-bearing coal was added, and a new clean resin froth was thus formed, which was removed in the usual manner.

The following table shows the results of four tests:

|                                  | Test #1<br>% wt. | Test #2<br>% wt. | Test #3<br>% wt. | Test #4<br>% wt. |
|----------------------------------|------------------|------------------|------------------|------------------|
| Resin coal                       | 100.0            | 100.0            | 100.0            | 100.0            |
| Resin 98% pure froth concentrate | 7.2              | 7.0              | 7.1              | 6.9              |
| Tailing—Coal residue             | 92.8             | 93.0             | 92.9             | 93.1             |

10 After the removal of the resin by froth flotation, the coal tailing or residue can be used directly as powdered coal fuel.

What I claim is:

15 1. The method of effecting separation of resin from resin-bearing coal, which comprises comminuting such coal and forming a pulp thereof, adding to such pulp a frothing agent that has a greater affinity for resin than for coal and subjecting the same to froth flotation treatment such frothing agent being used in quantity sufficient to float most of the resin but insufficient to float much of the coal.

20 2. The method of recovering resin from resin-bearing coal, which consists in comminuting such coal and forming a pulp thereof, adding to such pulp a flotation agent of the class which includes higher alcohol, turpentine, cresol and pine oil, in the proportion of about six-tenths of a pound of such flotation agent to a ton of coal and subjecting the pulp to froth flotation treatment.

25 3. The method of effecting separation of resin from resin-bearing coal, which comprises comminuting such coal and forming a pulp thereof, adding amyl alcohol to such pulp in the proportion of about six-tenths of a pound of amyl alcohol to a ton of coal and subjecting the same to froth flotation treatment.

40 4. The method of effecting separation of resin from resin-bearing coal, which comprises comminuting such coal and forming a pulp thereof, adding a frothing agent to such pulp and subjecting the same to froth flotation treatment to form a resin froth, placing said froth in a flotation machine, adding to the froth sufficient water to fill the flotation machine to working level together with about four-tenths of a pound of potassium alum per ton of original coal, agitating the same, and then adding about two-tenths of a pound of amyl alcohol per ton of resin bearing coal and subjecting the mixture to froth flotation.

45 5. The method of recovering resin from resin-bearing coal, which consists in comminuting such coal and forming a pulp thereof, adding to such pulp a flotation agent of the class which includes higher alcohol, turpentine, cresol and pine oil, in the proportion of about six-tenths of a pound of such flotation agent to a ton of coal and subjecting the pulp to froth flotation treatment to form a resin froth, placing said froth in a flotation machine, adding to the froth sufficient water to fill the flotation machine to working level to-

gether with about four-tenths of a pound of potassium alum per ton of original coal, agitating the same, and then adding about two-tenths of a pound of amyl alcohol per ton of resin bearing coal and subjecting the mixture to froth flotation.

6. The method of effecting separation of resin from resin-bearing coal, which comprises comminuting such coal and forming a pulp thereof, adding amyl alcohol to such pulp in the proportion of about six-tenths of a pound of amyl alcohol to a ton of coal and subjecting the same to froth flotation treatment to form a resin froth, placing said froth in a flotation machine, adding to the froth sufficient water to fill the flotation machine to working level together with about four-tenths of a pound of potassium alum per ton of original coal, agitating the same, and then adding about two-tenths of a pound of amyl alcohol per ton of resin bearing coal and subjecting the mixture to froth flotation.

7. The method of recovering resin from resin-bearing coal which consists in forming such coal into a water pulp and subjecting the same to ordinary froth flotation treatment to form a resin froth, forming said froth into a pulp by adding water thereto together with potassium alum in the proportion of about six-tenths of a pound thereof to a ton of the original coal and agitating the same, and then adding a fresh supply of frothing agent in the proportion of about two hundredths of one percent thereof to a ton of the original coal and forming a new resin froth.

8. The method of effecting separation of resin from resin-bearing coal which comprises comminuting such coal and forming a pulp thereof, adding suitable flotation agents to such pulp and subjecting the same to froth flotation treatment to form a resin froth, removing such froth from the original flotation machine, adding to such resin froth a depressant for coal, agitating the mixture of froth and coal depressant with suitable quantity of water then adding a frothing agent and subjecting the mixture to froth flotation treatment.

9. In the method of effecting separation of resin from resin-bearing coal by froth flotation, the improvement which consists in adding a coal depressant and a frothing agent to the pulp and then floating the resin.

Signed at Stockton, Utah, this 12th day of April, 1929.

WILLIAM D. GREEN.

120

125

130